



US005288598A

**United States Patent [19]**

Sterman et al.

[11] Patent Number: **5,288,598**[45] Date of Patent: **Feb. 22, 1994****[54] PHOTOGRAPHIC LIGHT-SENSITIVE ELEMENTS****[75] Inventors:** **Melvin D. Sterman**, Pittsford; **Alfred B. Fant**, Rochester; **Melvin M. Kestner**, Hilton; **Dennis E. Smith**; **Gary W. Visconte**, both of Rochester, all of N.Y.**[73] Assignee:** **Eastman Kodak Company**, Rochester, N.Y.**[21] Appl. No.:** **968,720****[22] Filed:** **Oct. 30, 1992****[51] Int. Cl.5** ..... **G03C 1/815****[52] U.S. Cl.** ..... **430/496; 430/523; 430/539; 430/536; 430/531; 430/627; 430/628; 430/950; 430/961****[58] Field of Search** ..... **430/496, 523, 539, 536, 430/531, 627, 628, 950, 961****[56] References Cited****U.S. PATENT DOCUMENTS**

|           |         |                  |          |
|-----------|---------|------------------|----------|
| 2,932,629 | 4/1960  | Wiley            | 526/226  |
| 2,976,250 | 3/1961  | Walford          | 430/523  |
| 3,206,312 | 9/1965  | Sterman et al.   | 430/529  |
| 3,411,907 | 11/1968 | Whitmore et al.  | 430/950  |
| 3,428,451 | 2/1969  | Trevoy           | 430/63   |
| 3,920,456 | 11/1975 | Nittel et al.    | 430/523  |
| 4,022,622 | 5/1977  | Timmerman et al. | 430/536  |
| 4,148,741 | 4/1979  | Bayley           | 252/62.1 |
| 4,203,769 | 5/1980  | Guestaux         | 430/631  |
| 4,232,117 | 11/1980 | Naoi et al.      | 430/539  |
| 4,232,117 | 11/1980 | Naoi et al.      | 430/539  |

|           |         |                   |         |
|-----------|---------|-------------------|---------|
| 4,235,959 | 11/1980 | Thijs et al.      | 430/531 |
| 4,264,707 | 4/1981  | Uozumi et al.     | 430/275 |
| 4,264,719 | 4/1981  | Kameoka et al.    | 430/950 |
| 4,275,103 | 6/1981  | Tsubasaki et al.  | 430/67  |
| 4,394,441 | 7/1983  | Kawaguchi et al.  | 430/524 |
| 4,396,706 | 8/1983  | Ishii et al.      | 430/403 |
| 4,409,322 | 10/1983 | Ezaki et al.      | 430/523 |
| 4,495,276 | 1/1985  | Takimoto et al.   | 430/527 |
| 4,524,131 | 6/1985  | Himmelmann et al. | 430/523 |
| 4,833,060 | 5/1989  | Nair et al.       | 430/137 |
| 4,833,060 | 5/1989  | Nair et al.       | 430/137 |
| 4,857,443 | 8/1989  | Aono et al.       | 430/496 |
| 4,868,088 | 9/1989  | Aono et al.       | 430/950 |
| 4,885,219 | 12/1989 | Miller            | 429/99  |
| 4,914,012 | 4/1990  | Kawai             | 430/536 |
| 4,975,363 | 12/1990 | Cavallo et al.    | 430/637 |
| 4,980,267 | 12/1990 | Taber             | 430/382 |
| 4,999,276 | 3/1991  | Kuwabara et al.   | 430/264 |
| 5,057,407 | 10/1991 | Okamura et al.    | 430/531 |

**OTHER PUBLICATIONS**

Research Disclosure 17643, Dec. 1978.

Research Disclosure 22534, Jan. 1983.

*Primary Examiner*—Charles L. Bowers, Jr.*Assistant Examiner*—Thomas R. Neville*Attorney, Agent, or Firm*—Robert A. Gerlach**[57] ABSTRACT**

Photographic elements containing at least one layer containing polymeric particles surrounded by a layer of colloidal inorganic particles and separate particles of colloidal silica.

**12 Claims, No Drawings**

## PHOTOGRAPHIC LIGHT-SENSITIVE ELEMENTS

## BACKGROUND OF THE INVENTION

## 1. Field of the Invention

This invention relates to silver halide photographic light-sensitive elements and more particularly to a method of forming images wherein the silver halide photographic light-sensitive element contains matting agents.

10 Finely divided materials with a mean particle size of from about 1 to about 10 micrometers are commonly used as matting agents to provide a rough surface to photographic elements. See, for example, U.S. Pat. Nos. 4,885,219 and 4,022,622. Further, U.S. Pat. Nos. 4,396,706 and 5,057,407 provide matte particles and techniques in order to increase the adhesion of the particles to the photographic element during processing of the element. In addition to the problems expressed in the previously recited references, printer dusting is also an objectionable problem associated with inadequate matte adhesion.

15 It has been heretofore known to use silica particles having a average particle size of 1 to 10 micrometers as mattes for use in photographic elements. In this regard, note U.S. Pat. Nos. 4,022,622; 2,976,250; 3,920,456; 4,409,322; and 4,396,706. The use of silica particles as mattes for use in photographic elements suffer from a number of disadvantages: they produce an objectionable, slightly milky appearance, their average grain size cannot be closely controlled, they adhere to wall surfaces and therefore give rise to extensive cleaning of equipment and increased labor costs and they settle out in the coating device and supply pipes, thus rendering impossible the precise metering of given quantities to the coating formulation. In addition to the above, the use of colloidal silica in conjunction with matte is disclosed in U.S. Pat. Nos. 4,975,363; 4,914,012; and 4,232,117.

20 U.S. Pat. No. 4,235,959 suggests the use of matte particles prepared by condensing in an aqueous medium urea and formaldehyde while vigorously stirring the mixture until particles comprising urea-formaldehyde resin and silica are formed wherein the silica is embedded within the resin matrix.

## SUMMARY OF THE INVENTION

The invention contemplates a photographic element having at least one light-sensitive layer on a support, the light-sensitive element containing a layer containing a first particulate material and a second particulate material, the first particulate material being polymer matte particles surrounded by a layer of colloidal inorganic particles and the second particulate material, being colloidal silica. The matte particles or beads in accordance with this invention can be included in any layer of the photographic element, but preferably are included in the top most surface of a light-sensitive silver halide photographic element, in a separate layer over the top surface of the photographic element or in a layer in close proximity to the top-most layer so that, the matte particles protrude above the surface of the top-most layer. The matte particles are included in a suitable binder such as gelatin and the like. The polymeric matte particles which are surrounded by a layer of colloidal inorganic particles have a mean diameter ranging from about 0.5 to about 10 and preferably from about 0.5 to about 5 micrometers and most preferably from about 1 to about 3.5 micrometers. The colloidal inorganic parti-

cles of the first particulate material and the colloidal silica of the second particulate material each has a particle diameter less than 50 nm and preferably from about 10 to about 25 nm.

5 Photographic elements in accordance with this invention demonstrate improved processing characteristics in modern rapid development apparatus with respect to matte adhesion, printer dusting, lack of haze and improved back side abrasion.

## DETAILED DESCRIPTION OF THE INVENTION

The matte particles of the first particulate material in accordance with this invention include a polymeric core material surrounded by a layer of colloidal inorganic particles.

10 Any suitable colloidal inorganic particles can be used to form the particulate layer on the polymeric core, such as, for example, silica, alumina, alumina-silica, tin oxide, titanium dioxide, zinc oxide and the like. Colloidal silica is preferred for several reasons including ease of preparation of the coated polymeric particles and improved adhesion of the matte particles to the photographic element during processing. For the purpose of simplification of the presentation of this invention, throughout the remainder of this specification colloidal silica will be used as the "colloidal inorganic particles" surrounding the polymeric core material, however, it should be understood that any of the colloidal inorganic particles may be employed.

15 Any suitable polymeric material or mixture of polymeric materials capable of being formed into particles having the desired size may be employed in the practice of this invention to prepare matte particles for use in photographic elements, such as, for example, olefin homopolymers and copolymers, such as polyethylene, polypropylene, polyisobutylene, polyisopentylene and the like; polyfluoroolefins such as polytetrafluoroethylene, polyvinylidene fluoride and the like, polyamides, such as, polyhexamethylene adipamide, polyhexamethylene sebacamide and polycaprolactam and the like; acrylic resins, such as polymethylmethacrylate, polyacrylonitrile, polymethylacrylate, polyethylmethacrylate and styrene-methylmethacrylate or ethylene-methyl acrylate copolymers, ethylene-ethyl acrylate copolymers, ethylene-ethyl methacrylate copolymers, polystyrene and copolymers of styrene with unsaturated monomers mentioned below, polyvinyltoluene, 20 cellulose derivatives, such as cellulose acetate, cellulose acetate butyrate, cellulose propionate, cellulose acetate propionate, and ethyl cellulose; polyvinyl resins such as polyvinyl chloride, copolymers of vinyl chloride and vinyl acetate and polyvinyl butyral, polyvinyl alcohol, polyvinyl acetal, ethylene-vinyl acetate copolymers ethylene-vinyl alcohol copolymers, and ethylene-allyl copolymers such as ethylene-allyl alcohol copolymers, ethylene-allyl acetone copolymers, ethylene-allyl benzene copolymers ethylene-allyl ether copolymers, ethylene-acrylic copolymers and polyoxy-methylene, polycondensation polymers, such as, polyesters, including polyethylene terephthalate, polybutylene terephthalate, polyurethanes and polycarbonates.

25 As indicated above, the most preferred mean particle size of the polymeric particles is from about 1 to about 3.5 micrometers. The mean diameter is defined as the mean of volume distribution. For best results, the polymeric particles should be less than 5,000 parts per mil-

lion of particles having a diameter greater than about 5 micrometers and less than 300 parts per million of particles having a diameter greater than about 8 micrometers.

Any suitable method of preparing polymeric particles surrounded by a layer of colloidal silica may be used to prepare the matte bead particles for use in accordance with this invention. For example, suitably sized polymeric particles may be passed through a fluidized bed or heated moving or rotating fluidized bed of colloidal silica particles, the temperature of the bed being such to soften the surface of the polymeric particles thereby causing the colloidal silica particles to adhere to the polymer particle surface. Another technique suitable for preparing polymer particles surrounded by a layer of colloidal silica is to spray dry the particles from a solution of the polymeric material in a suitable solvent and then before the polymer particles solidify completely, passing the particles through a zone of colloidal silica wherein the coating of the particles with a layer of the colloidal silica takes place. Another method to coat the polymer particle with a particulate layer of colloidal silver or by Mechano Fusion.

A still further method of preparing the matte particles in accordance with this invention is by limited coalescence. This method includes the "suspension polymerization" technique and the "polymer suspension" technique. In the "suspension polymerization" technique, a polymerizable monomer or monomers are added to an aqueous medium containing a particulate suspension of colloidal silica to form a discontinuous (oil droplets) phase in a continuous (water) phase. The mixture is subjected to shearing forces by agitation, homogenization and the like to reduce the size of the droplets. After shearing is stopped, an equilibrium is reached with respect to the size of the droplets as a result of the stabilizing action of the colloidal silica stabilizer in coating the surface of the droplets and then polymerization is completed to form an aqueous suspension of polymer particles in an aqueous phase having a uniform layer thereon of colloidal silica. This process is described in U.S. Pat. Nos. 2,932,629 and 4,148,741 incorporated herein by reference.

In the "polymer suspension" technique, a suitable polymer is dissolved in a solvent and this solution is dispersed as fine water-immiscible liquid droplets in an aqueous solution that contains colloidal silica as a stabilizer. Equilibrium is reached and the size of the droplets is stabilized by the action of the colloidal silica coating the surface of the droplets. The solvent is removed from the droplets by evaporation or other suitable technique resulting in polymeric particles having a uniform coating thereon of colloidal silica. This process is further described in U.S. Pat. No. 4,833,060 issued May 23, 1989, assigned to the same assignee as this application herein incorporated by reference.

In practicing this invention, using the suspension polymerization technique, any suitable monomer or monomers may be employed such as, for example, styrene, vinyl toluene, p-chlorostyrene; vinyl naphthalene; ethylenically unsaturated mono olefins such as ethylene, propylene, butylene and isobutylene; vinyl halides such as vinyl chloride, vinyl bromide, vinyl fluoride, vinyl acetate, vinyl propionate, vinyl benzoate and vinyl butyrate; esters of aliphatic acids such as methyl acrylate, ethyl acrylate, n-butylacrylate, isobutyl acrylate, dodecyl acrylate, n-octyl acrylate, 2-chloroethyl acrylate,

phenyl acrylate, methyl-alpha-chloroacrylate, methyl methacrylate, ethyl methacrylate and butyl methacrylate; acrylonitrile, methacrylonitrile, acrylamide, vinyl ethers such as vinyl methyl ether, vinyl isobutyl ether and vinyl ethyl ether; vinyl ketones such as vinyl methylketone, vinyl hexyl ketone and methyl isopropyl ketone; vinylidene halides such as vinylidene chloride and vinylidene chlorofluoride; and N-vinyl compounds such as N-vinyl pyrrole, N-vinyl carbazole, N-vinyl indole and N-vinyl pyrrolidone; divinyl benzene, ethylene glycol dimethacrylate, mixtures thereof, and the like.

In the suspension polymerization technique, other addenda are added to the monomer droplets and to the aqueous phase of the mass in order to bring about the desired result including initiators, promoters and the like which are more particularly disclosed in U.S. Pat. Nos. 2,932,629 and 4,148,741, both of which are incorporated herein in their entirety.

Useful solvents for the polymer suspension process are those that dissolve the polymer, which are immiscible with water and which are readily removed from the polymer droplets such as, for example, chloromethane, dichloromethane, ethylacetate, vinyl chloride, methyl ethyl ketone, trichloromethane, carbon tetrachloride, ethylene chloride, trichloroethane, toluene, xylene, cyclohexanone, 2-nitropropane and the like. A particularly useful solvent is dichloromethane because it is a good solvent for many polymers while at the same time, it is immiscible with water. Further, its volatility is such that it can be readily removed from the discontinuous phase droplets by evaporation.

The quantities of the various ingredients and their relationship to each other in the polymer suspension process can vary over wide ranges, however, it has generally been found that the ratio of the polymer to the solvent should vary in an amount of from about 1 to about 80% by weight of the combined weight of the polymer and the solvent and that the combined weight of the polymer and the solvent should vary with respect to the quantity of water employed in an amount of from about 25 to about 50% by weight. The size and quantity of the colloidal silica stabilizer depends upon the size of the particles of the colloidal silica and also upon the size of the polymer/solvent droplets desired. Thus, as the size of the polymer/solvent droplets are made smaller by high shear agitation, the quantity of solid colloidal stabilizer is varied to prevent uncontrolled coalescence of the droplets and to achieve uniform size and narrow size distribution of the polymer particles that result. The suspension polymerization technique and the polymer suspension technique herein described are the preferred methods of preparing the matte particles having a uniform layer of colloidal silica thereon for use in the preparation of light-sensitive photographic elements in accordance with this invention. These techniques provide particles having a predetermined average diameter anywhere within the range of from 0.5 micrometer to about 150 micrometers with a very narrow size distribution.

The coefficient of variation (ratio of the standard deviation to the average diameter, as described in U.S. Pat. No. 2,932,629, referenced previously herein, are normally in the range of about 15 to 35%.

The second particulate material is colloidal silica. Colloidal silica particles are small, discrete and uniformly dispersed in water alkaline media which reacts with the silica surface to produce a negative charge on the particles that repel each other to make up a stable

water dispersion. A suitable dispersion is one sold under the trade designation Ludox by DuPont Co. While the use of colloidal inorganic particle coated polymeric particles in accordance with U.S. Ser. No. 07/968,801, assigned to the same assignee as this application, filed on even date herewith establishes an improved and unexpected adhesion to photographic film during and after passage through modern automatic film processing apparatus, the further improvement in adhesion by combining such particles with colloidal silica particles as a second particulate material is quite unexpected.

The mattes made in accordance with this invention strongly adhere to the film thus eliminating the problems of processing solutions scumming and printer dusting. Also, the matting agents in accordance with the invention have unexpectedly improved backside abrasion such as that generally observed when silica mattes are employed.

In this invention, the matting agent is generally incorporated into the outermost layer of a light sensitive material, however, as indicated above, the matting agent can be incorporated into any layer of the light sensitive element. By outermost layer is meant either the emulsion side surface protecting layer or a backing layer or both. However, it is particularly preferable to incorporate the matting agent in the surface protecting layer.

Another advantage of the matting agents of this invention is that equipment such as, dissolution tanks and the like used in the process of production are washed with ease because the matting agent does not adhere firmly to the wall surfaces.

The matting agents are employed in an amount to achieve a coverage of from about 2 to about 500 mg per square meter. The matte particle content should range from 0.3 to 25 weight percent of the gelatin content of the layer and preferably from about 0.6 to 18.5 weight percent. The colloidal silica preferably should be employed in an amount up to about 50 weight percent based on the gelatin content of the layer and preferably in an amount of from about 5 to about 40 percent by weight.

Should the matte particles be incorporated in a separate overcoat protective layer, any suitable binder may be used, such as, gelatin, polymers and the like.

As for gelatin, any kinds of gelatin, for example, alkali-processed gelatin, acid-processed gelatin, enzyme-processed gelatin, gelatin derivatives and denatured gelatins are usable.

Further, the outermost layer of this invention may optionally contain a hardening agent, a smoothing agent, a surface active agent, an antistatic agent, a thickener, polymers, an ultraviolet ray absorbent, a high boiling point solvent, silver halides, a formalin capturing agent, a polymer latex and various other additives.

Examples of a hardening agent employable in this invention includes aldehyde series compounds, active halogen-containing compounds such as 2-hydroxy-4,6-dichloro-1,3,5-triazine, vinyl sulfone series compounds, N-methylol series compounds, halogencarboxyaldehyde compounds such as mucochloric acid, and so on.

As a surface active agent, any kind of surface active agents, for example, natural surface active agents such as saponin, nonionic surface active agents such as polyalkyleneoxides, cationic surface active agents such as higher alkylamines, quaternary ammonium salts and so on; anionic surface active agents containing acidic

groups such as carboxylic acid, sulfonic acid and so forth, may be employed.

As an antistatic agent, the outermost layer may contain surface active agents as described above, alkali metal salts of styrene-maleic acid series copolymers and acrylonitrile-acrylic acid series copolymers, and antistatic agents as described in U.S. Pat. Nos. 3,206,312; 3,428,451; metal oxides, such as  $V_2O_5$ ,  $SnO_2$ , antimony doped  $SnO_2$ ,  $ZnO_2$ ,  $TiO_2$  and the like. Suitable metal oxides are set forth in U.S. Pat. Nos. 4,203,769; 4,264,707; 4,275,103; 4,394,441; 4,495,276; 4,999,276 and so forth.

Photographic elements in which the particles of the invention can be utilized generally comprise at least one light-sensitive layer, such as a silver halide emulsion layer. This layer may be sensitized to a particular spectrum of radiation with, for example, a sensitizing dye, as is known in the art. Additional light-sensitive layers may be sensitized to other portions of the spectrum. The light sensitive layers may contain or have associated therewith dye-forming compounds or couplers. For example, a red-sensitive emulsion would generally have a cyan coupler associated therewith, a green-sensitive emulsion would be associated with a magenta coupler, and a blue-sensitive emulsion would be associated with a yellow coupler. Other layers and addenda, such as antistatic compositions, subbing layers, surfactants, filter dyes, protective layers, barrier layers, development inhibiting releasing compounds, and the like can be present in photographic elements of the invention, as is well-known in the art. Detailed description of photographic elements and their various layers and addenda can be found in the above-identified *Research Disclosure* 17643 and in James, *The Theory of the Photographic Process*, 4th, 1977.

Photographic elements suitable for use in combination with the overcoat layer containing matte particles in accordance with this invention are disclosed in *Research Disclosure* 22534, January 1983, which is incorporated herein by reference. Further, the light sensitive elements disclosed in U.S. Pat. No. 4,980,267 fully incorporated herein by reference are particularly applicable to protection by the overcoat layers in accordance with this invention.

It is, at times, desirable to include in the layer containing the matte particles in accordance with this invention, an amount of polymeric emulsion polymerized latex particles to improve adhesion during processing. Suitable polymeric latex particles have a diameter of from about 0.01 to 0.5  $\mu$ m, preferably from about 0.02 to about 0.1  $\mu$ m and are employed in an amount of from about 10 to about 75 weight percent, preferably from about 25 to about 50 percent by weight based on the weight of the gelatin present in the layer. Suitable monomers for use in the preparation of latex homopolymers or copolymers include, for example, methyl acrylate, methyl methacrylate, 2-acrylamido-2-methyl propane sulfonic acid, styrene, butyl methacrylate, 2-methacryloyloxyethyl-1-sulfonic acid-sodium salt, vinylidene chloride, itaconic acid, acrylonitrile, acrylic acid, n-butyl acrylate, 2-[N,N,N-trimethyl ammonium] ethyl methacrylate methosulfate and the like. Particularly, suitable copolymers include polymethyl acrylate-co-2-acrylamido-2-methylpropane sulfonic acid (96:4), styrene-co-butylmethacrylate-co-2-methacryloyloxyethyl-1-sulfonic acid-sodium salt, methyl acrylate-co-vinylidene chloride-co-itaconic acid, acrylonitrile-co-vinylidene chloride-co-acrylic acid, n-butyl acrylate-

co-methylmethacrylate, acrylonitrile-co-vinylidene chloride-co-2[N,N,N,bimethyl ammonium] ethyl methacrylate methosulfate and the like.

It is also, at times, desirable to employ as the polymer for the matte particles one that has a refractive index that closely matches that of the binder for the layer containing the particles. For example, if gelatin is the binder, a polymer or copolymer having a refractive index as close to 1.54, as possible, will result in improved light transmission of the layer and thus improved characteristics for the photographic element.

The invention is further illustrated by the following examples:

#### EXAMPLE 1

##### Preparation of Colloidal Silica Coated Vinyl Toluene Particles

15 g of Vazo 67 sold by DuPont Co. are dissolved in 1500 g of vinyltoluene. In a separate container, 2500 g of distilled water are added. To the water, 0.45 g potassium dichromate, 31 g poly(2-methylaminoethanol) adipate (MAEA) and 275 g Ludox TM (colloidal silica, particle size 21nm, sold by DuPont Co.) are added. The monomer solution is combined with the aqueous solution and stirred for 10 minutes. A Gaulin homogenizer at 3000 psi is used to form the emulsion. The emulsion is reacted at 70° C. for a time period of 20 hours using a constant agitation of 125 RPM. Beads are then filtered and washed to remove potassium dichromate. This procedure yields a mean volume size particle of 2.9 microns.

#### EXAMPLE 2

##### Photographic Element

A series of color photographic elements are prepared as follows:

A cellulose triacetate film support having an antihalation layer on one side and an antistatic layer on the other side is coated on the antihalation layer with the following layers in sequence (coverages are in grams per meter squared):

##### Slow Cyan Dye-Forming Layer

This layer comprises a blend of red-sensitized, cubic, silver bromoiodide emulsion (1.5 mole percent iodide) (0.31 um grain size) (1.16 g/m<sup>2</sup>) and red sensitized, tabular grain, silver bromoiodide emulsion (3 mole percent iodide) (0.75 um diameter by 0.14 um thick) (1.31), Compound J (0.965), Compound E (0.011), Compound L (0.65) and gelatin (2.96).

##### Fast Cyan Dye-Forming Layer

This layer comprises a red sensitized, tabular grain silver bromoiodide emulsion (6 mole percent iodide)

having a diameter of 1.4 um and a thickness of 0.12 um (0.807), Compound J (0.102), Compound K (0.065), Compound L (0.102) and gelatin (1.506).

##### Interlayer

This layer comprises Compound F (0.054), an anti-fogger and gelatin (1.291)

##### Slow Magenta Dye-Forming Layer

This layer comprises a blend of green-sensitized tabular grain silver bromoiodide emulsion (3 mole percent iodide) (grain diameter 0.55 um and thickness 0.08 um) (0.473) and tabular grain silver bromoiodide emulsion (3 mole percent iodide) (grain diameter 0.52 and thickness 0.09 um) (0.495), Compound g (0.161), Compound I (0.108) and gelatin (2.916).

##### Fast Magenta Dye-Forming Layer

This layer comprises a blend of green-sensitized tabular grain silver bromoiodide emulsion (3 mole percent iodide) (grain diameter 1.05 um and thickness 0.12 um) (0.536) and tabular grain silver bromoiodide emulsion (3 mole percent iodide) (grain diameter 0.75 um and thickness 0.14 um, Compound G (0.258), Compound H (0.054) and gelatin (1.119).

##### Interlayer

This layer comprises Carey-Lea Silver (0.43), Compound F (0.054), an antifogger and gelatin (0.861).

##### Slow Yellow Dye-Forming Layer

This layer comprises a blend of blue-sensitized tabular grain silver bromoiodide emulsions (3 mole percent iodide) (grain diameter 0.57 um and thickness 0.12 um) (0.274) and blue sensitive silver bromoiodide emulsion (0.3 mole percent iodide) (grain diameter 0.52 um and thickness 0.09 um) (0.118), Compound C (1.022), Compound D (0.168) and gelatin (1.732).

##### Fast Yellow Dye-Forming Layer

This layer comprises a blue-sensitized tabular grain silver bromoiodide emulsion (3 mole percent iodide) (grain diameter 1.10 um and thickness 0.12 um) (0.43), Compound C (0.161), Compound D (0.054), Compound E (0.003) and gelatin (0.791). cl UV Absorbing Layer

This layer comprises silver halide Lippmann emulsion (0.215), Compound A (0.108), Compound B (0.106) and gelatin (0.538).

##### Overcoat

This layer comprises matte particles of Example 1 (0.038) and gelatin (0.888).

The structures of the above-designated compounds A through L are as follows:



-continued



-continued



(A) The coating solution for the gelatin overcoat is 60 prepared in the following manner:

In a mixing vessel combine 1179 grams of Type IV gelatin, as a swollen gelatin which contains 65% water, 1000 grams distilled water, 285.3 grams of a matte dispersion, which consists of 6.75% poly(vinyl toluene) 65 matte beads, 7.5% Type IV gelatin, and the balance being distilled water, and 222 grams of a lubricant/gelatin dispersion which contains 9.0% Type IV gelatin.

This mixture is heated at 46° C. with gentle stirring until the gelatin has dissolved completely, approximately 30 minutes, and a uniform solution is achieved.

This solution is held at 46° C. and the following addenda are added in the following order:

|                |                          |
|----------------|--------------------------|
| Sulfuric acid  | 30 cc/pound gelatin      |
| Alkanol XC     | 13.6 cc/pound of gelatin |
| Surfactant 10G | 14.9 cc/pound of gelatin |

|               |                      |
|---------------|----------------------|
| Fluorad FC135 | 2.0 cc/pound gelatin |
|---------------|----------------------|

This solution is then cooled to 40° C.; the pH adjusted to 5.5 with either a weak acid or base as needed and distilled water added to bring the total weight of the solution to 4761.0 grams.

This coating solution is applied to the photographic element described.

(B) A solution is prepared as described in (A) except that in addition colloidal silica (Ludox AM, supplied by DuPont Co., particle size 12nm) is added in an amount equal to 33 percent by weight of the gelatin content of the solution and applied to the element in the same manner.

(C) A solution is prepared as described in (A) except that the poly(vinyl toluene) matte beads are replaced with poly(vinyl toluene) matte beads as prepared in Example 1. This solution is coated as indicated above.

(D) A solution is prepared and coated as described in (C) except that in addition colloidal silica (Ludox AM) is added in an amount equal to 33 weight percent of the gelatin content of the solution.

(E) A solution is prepared and coated as described in (B) except that the poly(vinyl toluene) matte beads are replaced with poly(vinyl toluene-co-methyl methacrylate) matte beads, wherein the vinyl toluene content is 40 weight percent and the methylmethacrylate content is 60 weight percent and there is outer shell of 21 nanometer diameter silica particles on the surface of the polymer beads. These particles are prepared in accordance with the procedure of Example 1 except for substitution of the starting comonomers for the vinyl toluene of (B).

(F) A solution is prepared and coated as described in (E) except that the monomer content of the matte beads is 50 weight percent vinyl toluene and 50 weight percent methyl methacrylate.

(G) (Control) A solution is prepared and coated as described in (F) except that the matte beads did not have an outer shell of silica on the surface of the polymer beads.

(H) A solution is prepared and coated as described in (E) except that the monomer content of the matte beads is 60 percent vinyl toluene and 40 weight percent methyl methacrylate.

(I) A solution is prepared and coated as described in (E) except that the polyvinyl toluene-co-methyl methacrylate matte beads are replaced with poly(vinyl toluene-co-tert-butyl styrene) matte beads, wherein the vinyl toluene content is 95 weight percent and the tert-butyl styrene content is 5 weight percent, and there is an outer shell of 21 nanometer silica particles on the surface of the polymer beads. The matte particles are prepared in a similar manner to that described in Example 1.

(J) A solution is prepared and coated as described in (E) except that the polyvinyl toluene-co-methyl methacrylate matte beads are replaced with poly(methyl methacrylate-co-tert-butyl styrene) matte beads, wherein the methyl methacrylate content is 95 weight percent and the tert-butyl styrene content is 5 weight percent, and there is an outer shell of 21 nanometer silica particles on the surface of the polymer beads. The matte particles are prepared in a similar manner to that described in Example 1.

(K) A solution is prepared as described in (E) except that the polyvinyl toluene-co-methyl methacrylate matte beads are replaced with poly(methyl methacrylate) matte beads which have an outer shell of 21 nanometer silica particles on the surface of the polymer beads. The particles are prepared in a similar manner to that described in Example 1.

(L) A solution is prepared and coated as described in (B) except that the poly(vinyl toluene) matte beads are replaced with poly(methyl methacrylate) matte beads.

#### EVALUATION METHODS

Equal footage of film from each of the experimental coatings is perforated for use in a 35 mm camera and exposed. These exposed films are then processed in a standard photofinishing processor with fresh stabilizer solution, which is the final solution in the process, to insure that the matte beads from previously processed films will not be deposited on the test film surface.

The processed films are then printed in a standard photofinishing high speed printer which has roller contact with the topmost protective layer of the film which contains the matte beads. Following the printing operation for each film sample, the roller is removed and analyzed for the number of matte beads that transfer to the roller, i.e., dusted from the film surface due to poor adhesion.

The films prepared in parts A, B, C and D of Example 2 are evaluated for matte adhesion by the above method and the results are reported in Table 1. These data demonstrate the very significant improvement in matte bead retention, or conversely, the reduction in matte bead loss observed with those film samples in which colloidal silica is present as an addendum in the topmost protective layer and the matte beads have a surface shell of silica particles.

In an alternative method of analysis, following the printing operation, each of the processed films is evaluated for matte adhesion by examining the surface of each film sample with an optical microscope and counting the number of craters, or pits, on the surface which result from the removal of matte beads during the processing, notching and printing operations. A constant surface area is used for each film sample in this procedure. This procedure is appropriate only when process surviving mattes are used.

The films prepared in Example 2 (A) through (L) are evaluated for matte adhesion by this method and the results are reported in Table 2. These data demonstrate the very significant improvement in matte bead retention which is observed in those film samples in which colloidal silica is present as an addendum in the topmost protective layer and the matte beads have a surface shell of silica particles.

The films prepared in Example 2 (A), (B), (C) and (D) are also evaluated for resistance to abrasion and scratching by the Taber Abrader test. This abrasion test is conducted on the processed emulsion using two wheels with a load of 185 grams for 100 cycles. The data are reported as the percent delta haze, i.e., the difference in haze of the test film sample measured before and after the abrader test. The higher the magnitude of the percent delta haze, the greater is the degree of abrasion to the film sample. The results of these measurements are also reported in Table 1. The significant reduction in abrasion and scratching observed in this test in film samples in which colloidal silica is present as an addendum

dum in the topmost protective layer is clearly demonstrated by these data.

TABLE 1

| Example 1 | Colloidal Silica | PPCM | Actual Bead Count | Normalized Bead Count | Taber Abrasion Delta % Haze 2 wheels |
|-----------|------------------|------|-------------------|-----------------------|--------------------------------------|
| A         | None             | 84   | 784               | 9.33                  | 11.0                                 |
| B         | 33 wt %          | 86   | 813               | 9.45                  | 3.8                                  |
| C         | None             | 75   | 94                | 1.25                  | 6.8                                  |
| D         | 33 wt %          | 82   | 51                | 0.62                  | 3.0                                  |

PPCM = particles per centimeter measured by a stylus instrument.

Normalized Bead Count = (actual bead count/PPCM)  $\times 10$

TABLE 2

| Example 2 | Silica Shell | Matte Size (microns) | Colloidal Silica | Pit Count |
|-----------|--------------|----------------------|------------------|-----------|
| A         | No           | 3.2                  | None             | 137       |
| B         | No           | 3.2                  | 33 wt %          | 102/213   |
| C         | Yes          | 2.8                  | None             | 5         |
| D         | Yes          | 2.8                  | 33 wt %          | 1         |
| E         | Yes          | 2.3                  | 33 wt %          | 2         |
| F         | Yes          | 2.3                  | 33 wt %          | 28        |
| G         | No           | 1.2                  | 33 wt %          | 41        |
| H         | Yes          | 2.4                  | 33 wt %          | 15        |
| I         | Yes          | 1.8                  | 33 wt %          | 8         |
| J         | Yes          | 1.1                  | 33 wt %          | 41        |
| K         | Yes          | 2.5                  | 33 wt %          | 7         |
| L         | No           | 3.2                  | 33 wt %          | 486       |

It is, of course, to be understood that like materials can be substituted throughout these examples without departing from the spirit and scope of this invention.

What is claimed:

1. A photographic element comprising at least one light-sensitive layer on a support said element contain-

ing in at least one layer, a first particulate material and a second particulate material, said first particulate material being polymeric particles having a core surrounded by a shell of colloidal inorganic particles and said second particulate material being colloidal silica.

2. The photographic element of claim 1 wherein the polymeric particle core has a mean diameter of from 0.5 to 10 micrometers.

3. The photographic element of claim 1 wherein the polymeric particle core has a mean diameter of from 1 to 5 micrometers.

4. The photographic element of claim 1 wherein the polymeric particle core has a mean diameter of from 1 to 3.5 micrometers.

15 5. The photographic element of claim 1 wherein the polymeric particle core is a polyaddition polymer.

6. The photographic element of claim 1 wherein the polymeric particle core is a polycondensation polymer.

7. The photographic element of claim 4 wherein the polyaddition polymer is polyvinyltoluene.

8. The photographic element of claim 1 wherein the polymeric particles are included in the top-most layer.

9. The photographic element of claim 1 wherein the polymeric particles are included in an overcoat layer.

20 10. The photographic element of claim 1 wherein the second particulate material has a particle size of less than 50 nm.

11. The photographic element of claim 1 wherein the colloidal inorganic particles are colloidal silica, alumina, tin oxide, titanium dioxide, zinc oxide or mixtures thereof.

30 12. The photographic element of claim 11 wherein the colloidal inorganic particles are silica.

\* \* \* \* \*

35

40

45

50

55

60

65